



US005470664A

**United States Patent** [19]**Bartak et al.**[11] **Patent Number:** **5,470,664**[45] **Date of Patent:** **Nov. 28, 1995**[54] **HARD ANODIC COATING FOR MAGNESIUM ALLOYS**[75] Inventors: **Duane E. Bartak**, Cedar Falls, Iowa; **Brian E. Lemieux**, E. Grand Forks, Minn.; **Earl R. Woolsey**, Grand Forks, N. Dak.[73] Assignee: **Technology Applications Group**, Grand Forks, N. Dak.[21] Appl. No.: **271,052**[22] Filed: **Jul. 6, 1994**

|           |         |                   |       |          |
|-----------|---------|-------------------|-------|----------|
| 2,901,409 | 8/1959  | DeLong            | ..... | 204/56   |
| 3,732,152 | 5/1973  | Hawke             | ..... | 204/56 M |
| 3,791,942 | 2/1974  | McNeil            | ..... | 204/56 M |
| 3,832,293 | 8/1974  | Hradcovsky et al. | ..... | 204/56 R |
| 3,834,999 | 9/1974  | Hradcovsky et al. | ..... | 204/56 R |
| 3,956,080 | 4/1976  | Hradcovsky et al. | ..... | 204/56 R |
| 4,082,626 | 4/1978  | Hradcovsky        | ..... | 204/56 R |
| 4,184,926 | 1/1980  | Kozak             | ..... | 204/32 R |
| 4,592,958 | 6/1986  | Mosser et al.     | ..... | 428/432  |
| 4,620,904 | 11/1986 | Kozak             | ..... | 204/58.4 |
| 4,659,440 | 4/1987  | Hradcovsky        | ..... | 204/58   |
| 4,668,347 | 5/1987  | Habermann et al.  | ..... | 204/33   |
| 4,744,872 | 5/1988  | Kobayashi et al.  | ..... | 204/58.4 |
| 4,978,432 | 12/1990 | Schmeling et al.  | ..... | 204/58.4 |

*Primary Examiner*—Kathryn Gorgos*Assistant Examiner*—Kishor Mayekar*Attorney, Agent, or Firm*—Merchant, Gould, Smith, Edell, Welter & Schmidt[57] **ABSTRACT**

A two-step process for the coating of magnesium and its alloys is disclosed. The first step comprises immersing the magnesium workpiece in an aqueous solution comprising about 0.2 to 5 molar ammonium fluoride having a pH of about 5 to 8 and a temperature of about 40° to 100° C. The second step is an electrochemical treatment of the pretreated article in an aqueous electrolytic solution having a pH of at least about 12.5 and which solution comprises about 2 to 12 g/L of a aqueous soluble hydroxide, about 2 to 15 g/L of a fluoride-containing composition selected from the group consisting of fluorides and fluorosilicates, and about 5 to 30 g/L of a silicate. This process results in a superior coating which has increased abrasion and corrosion resistance.

**4 Claims, 2 Drawing Sheets**[56] **References Cited**

## U.S. PATENT DOCUMENTS

|           |         |             |       |         |
|-----------|---------|-------------|-------|---------|
| 1,574,289 | 2/1926  | Keeler      | ..... | 205/321 |
| 2,313,754 | 3/1943  | Loose       | ..... | 204/56  |
| 2,723,952 | 11/1955 | Evangelides | ..... | 204/35  |
| 2,766,199 | 10/1956 | Higgins     | ..... | 204/141 |
| 2,880,148 | 3/1959  | Evangelides | ..... | 204/35  |





FIG. 1



FIG. 2



FIG. 3



FIG. 4

## HARD ANODIC COATING FOR MAGNESIUM ALLOYS

### CROSS-REFERENCE TO RELATED APPLICATION

This application is a continuation-in-part of application Ser. No. 08/136,494 of Oct. 14, 1993, which is a continuation of application Ser. No. 07/869,427 of Apr. 16, 1992, now abandoned, which is a continuation of application Ser. No. 661,503 of Feb. 26, 1991, now abandoned.

### FIELD OF THE INVENTION

The invention relates to a process for forming a hard anodic coating on a magnesium alloy and to a product formed by this process. In particular, the invention relates to a method comprising pretreating an article comprising a magnesium alloy in a chemical bath at a neutral pH followed by an electrolytically coating the pretreated article in an aqueous solution.

### BACKGROUND OF THE INVENTION

The use of magnesium in structural applications is growing rapidly. Magnesium is generally alloyed with any of aluminum, manganese, thorium, lithium, tin, zirconium, zinc, rare earth metals or other alloys to increase its structural stability. Such magnesium alloys are often used where a high strength to weight ratio is required. The appropriate magnesium alloy can also offer the highest strength to weight ratio of the ultra light metals at elevated temperatures. Further, alloys with rare earth or thorium can retain significant strength up to temperatures of 315° C. and higher. Structural magnesium alloys may be assembled in many of the conventional manners including riveting and bolting, arc and electric resistance welding, braising, soldering and adhesive bonding. The magnesium-containing articles have uses in the aircraft and aerospace industries, military equipment, electronics, automotive bodies and parts, hand tools and in materials handling. While magnesium and its alloys exhibit good stability in the presence of a number of chemical substances, there is a need to further protect the metal, especially in acidic environments and in salt water conditions. Therefore, especially in marine applications, it is necessary to provide a coating to protect the metal from corrosion.

There are many different types of coatings for magnesium which have been developed and used. The most common coatings are chemical treatments or conversion coatings which are used as a paint base and provide some corrosion protection. Both chemical and electrochemical methods are used for the conversion of magnesium surfaces. Chromate films are the most commonly used surface treatment for magnesium alloys. These films of hydrated, gel-like structures of polychromates provide a surface which is a good paint base but which provides limited corrosion protection.

Anodization of magnesium alloys is an alternative electrochemical approach to provide a protective coating. At least two low voltage anodic processes, Dow 17 and HAE, have been commercially employed. However, the corrosion protection provided by these treatments remains limited. The Dow 17 process utilizes potassium dichromate, a chromium (VI) compound, which is acutely toxic and strictly regulated. Although the key ingredient in the HAE anodic coating is potassium permanganate, it is necessary to use a chromate sealant with this coating in order to obtain acceptable corrosion resistance. Thus in either case, chromium

(VI) is necessary in the overall process in order to achieve a desirable corrosion resistant coating. This use of chromium (VI) means that waste disposal from these processes is a significant problem.

More recently, metallic and ceramic-like coatings have been developed. These coatings may be formed by electroless or electrochemical processes. The electroless deposition of nickel on magnesium and magnesium alloys using chemical reducing agents in coating formulation is well known in the art. However, this process also results in the creation of large quantities of hazardous heavy metal contaminated waste water which must be treated before it can be discharged. Electrochemical coating processes can be used to produce both metallic and nonmetallic coatings. The metallic coating processes again suffer from the creation of heavy metal contaminated waste water.

Non-metallic coating processes have been developed, in part, to overcome problems involving the heavy metal contamination of waste water. Kozak, U.S. Pat. No. 4,184,926, discloses a two-step process for forming an anti-corrosive coating on magnesium and its alloys. The first step is an acidic chemical pickling or treatment of the magnesium work piece using hydrofluoric acid at about room temperature to form a fluoro-magnesium layer on the metal surface. The second step involves the electrochemical coating of the work piece in a solution comprising an alkali metal silicate and an alkali metal hydroxide. A voltage potential from about 150-300 volts is applied across the electrodes, and a current density of about 50-200 mA/cm<sup>2</sup> is maintained in the bath. The first step of this process is a straight forward acid pickling step, while the second step proceeds in an electrochemical bath which contains no source of fluoride. Tests of this process indicate that there is a need for increased corrosion resistance and coating integrity.

Kozak, U.S. Pat. No. 4,620,904, discloses a one-step method of coating articles of magnesium using an electrolytic bath comprising an alkali metal silicate, an alkali metal hydroxide and a fluoride. The bath is maintained at a temperature of about 5°-70° C. and a pH of about 12-14. The electrochemical coating is carried out under a voltage potential from about 150-400 volts. Tests of this process also indicates that there remains a need for increased corrosion resistance.

Based on the teachings of the prior art, a process for the coating of magnesium-containing articles is needed which results in a uniform coating with increased corrosion resistance. Further, a more economical coating process is needed which has reduced apparatus demands and which does not result in the production of heavy metal contaminated waste water.

### SUMMARY OF THE INVENTION

The present invention is directed to a process for coating a magnesium-containing article. The article is pretreated in an aqueous solution comprising about 0.2 to 5 molar ammonium fluoride having a pH of about 5 to 8 and a temperature of about 40° to 100° C. This pretreatment step cleans the article and creates a fluoride-containing layer, which is several hundred Angstroms thick at the surface of the article to form a pretreated article. Next, the pretreated article is immersed in an aqueous electrolytic solution having a pH of at least about 12.5 and which solution comprises about 2 to 12 g/L of a aqueous soluble hydroxide, about 2 to 15 g/L of a fluoride-containing composition selected from the group consisting of fluorides and fluorosilicates, and about 5 to 30

g/L of a silicate. A voltage differential of at least about 100 volts is established between an anode comprising the pre-treated article and a cathode also in contact with the electrolytic solution to create a current density of about 2 to 90 mA/cm<sup>2</sup>. Through this process, a magnesium oxide/silicon oxide-containing coating is formed on the magnesium-containing article.

The term "magnesium-containing article", as used in the specification and the claims, means a metallic article having surfaces which are in whole or in part metallic magnesium per se or a magnesium alloy. Preferably, the article is formed of metallic magnesium or a magnesium alloy and comprises a significant amount of magnesium. More preferably, the article comprises a magnesium-rich alloy comprising at least about 50 wt-% magnesium, and most preferably, the article comprises at least about 80 wt-% magnesium.

#### BRIEF DESCRIPTION OF THE DRAWINGS

FIG. 1 illustrates the coated magnesium-containing article of the invention.

FIG. 2 is a block diagram of the present invention.

FIG. 3 is a diagram of the electrochemical process of the invention.

FIG. 4 is a scanning electron photomicrograph of a cross section through the magnesium-containing substrate and a coating according to the invention.

#### DETAILED DESCRIPTION OF THE PREFERRED EMBODIMENT

FIG. 1 illustrates a cross section of a magnesium-containing article having been coated using the process of the present invention. The magnesium-containing article 10 has been masked off in areas 16 to provide a comparison of coated surface versus uncoated surface. The surface of the article exposed to the process of the present invention is shown with a coating 12 containing a composite of metal fluoride, metal oxide, and silicon oxide. The coating 12 forms a corrosion resistant coating on the surface of the magnesium-containing article. Coatings include ceramic-like, magnesium oxide/silicon oxide containing coatings.

FIG. 2 illustrates the steps used to produce these coated articles. An untreated article 20 is first placed in a chemical bath 22 which cleans and forms a fluoride-containing layer on the article. Next, the article is treated in an electrochemical bath 24 resulting in the production of a coated article 26.

The chemical bath 22 comprises an aqueous ammonium fluoride solution. Preferably, the bath comprises 0.2 to 5 molar ammonium fluoride in water, more preferably, 0.3 to 3.0 molar ammonium fluoride and, most preferably, about 2.0 to 3.0 molar ammonium fluoride. The reaction conditions are indicated below in Table I.

TABLE I

| Condition         | Preferred | More Preferred | Most Preferred |
|-------------------|-----------|----------------|----------------|
| pH                | 4-8       | 5-7            | 6-7            |
| Temperature (°C.) | 40-100    | 55-90          | 70-85          |
| Time (minutes)    | 15-60     | 30-45          | 30-40          |

If the bath is too acidic or too hot, too vigorous of an oxidation (etching) reaction occurs, and if the bath is too alkaline or too cool, the reaction proceeds too slowly for practical production of coated articles.

The magnesium-containing article is maintained in the chemical bath for a time sufficient to clean impurities at the surface of the article and to form a fluoride-containing base layer of several hundred Angstroms thick on the magnesium-containing article. This results in the production of a magnesium-containing article which is coated with predominately metal fluoride with small amounts of metal oxide and/or metal oxofluoride, most of the metal being magnesium depending on the nature of the alloy. Too brief a residence time in the chemical bath results in an insufficient fluoride containing base layer and/or insufficient cleaning of the magnesium-containing article. This will ultimately result in the reduced corrosion resistance of the coated article. Longer residence times tend to be uneconomical as the process time is increased with little improvement of the base layer. This base layer is generally uniform in composition and thickness across the surface of the article and provides an excellent base upon which a ceramic-like layer may be formed. Preferably, the thickness of this fluoride containing layer is greater than 1000 Angstroms.

While we do not wish to be confined to this theory, it appears that the first chemical bath is beneficial as it provides a base layer which firmly bonds to the substrate and which is compatible with the formation of a ceramic-like layer. It appears that the base layer comprises metal fluorides and oxofluorides which strongly adhere to the metallic substrate. It appears that the compatibility of these compounds with those of the ceramic-like layer permits the concurrent deposition of silicon oxide and formation of magnesium oxide among other compounds, in a uniform manner.

This base layer provides some protection to the metallic substrate, but it does not provide the abrasion resistance and hardness that the completely integrated coating provides. On the other hand, if the magnesium oxide/silicon oxide-containing layer is formed on the metallic substrate without first forming the base layer, the corrosion and abrasion resistance of the coating is reduced as the magnesium oxide/silicon oxide-containing layer does not adhere well to the substrate.

Between the chemical bath 22 and the electrochemical bath 24, the pretreated article is preferably thoroughly washed with water to remove any unreacted ammonium fluoride. This cleaning prevents the contamination of the electrochemical bath 24.

The cleaned, pretreated article is then subjected to an electrochemical coating process shown in FIG. 3. The electrochemical bath 24 comprises an aqueous electrolytic solution comprising about 2 to 12 g/L of a soluble hydroxide compound, about 2 to 15 g/L of a soluble fluoride-containing compound selected from the group consisting of fluorides and fluorosilicates and about 5 to 30 g/L of a silicate. Preferred hydroxides include alkali metal hydroxides. More preferably, the alkali metal is lithium, sodium or potassium, and most preferably, the hydroxide is potassium hydroxide.

The fluoride-containing compound may be a fluoride such as an alkali metal fluoride, such as lithium, sodium and

potassium fluoride or an acid fluoride such as hydrogen fluoride or ammonium bifluoride. Fluorosilicates such as potassium fluorosilicate or sodium fluorosilicate may also be used. Preferably, the fluoride-containing compound comprises an alkali metal fluoride, an alkali metal fluorosilicate, hydrogen fluoride or mixtures thereof. Most preferably, the fluoride-containing compound comprises potassium fluoride.

The electrochemical bath also contains a silicate. Useful silicates include alkali metal silicates and/or alkali metal fluorosilicates. More preferably, the silicate comprises lithium, sodium or potassium silicate, and most preferably, the silicate is potassium silicate.

Composition ranges for the aqueous electrolytic solution are shown below in Table II.

TABLE II

| Component | Preferred | More Preferred | Most Preferred |
|-----------|-----------|----------------|----------------|
| Hydroxide | 2-12 g/L  | 4-8 g/L        | 5-7 g/L        |
| Fluoride  | 2-15 g/L  | 3-10 g/L       | 8-10 g/L       |
| Silicate  | 5-30 g/L  | 10-25 g/L      | 15-20 g/L      |

The pretreated article 30 is immersed in the electrochemical bath 24 as an anode. The vessel 32 which contains the electrochemical bath 24 may be used as the cathode. The anode may be connected through a switch 34 to a rectifier 36 while the vessel 32 may be directly connected to the rectifier 36. The rectifier 36, rectifies the voltage from a voltage source 38, to provide a direct current source to the electrochemical bath. The rectifier 36 and switch 34 may be placed in communication with a microprocessor control 40 for purposes of controlling the electrochemical composition. Preferably, the rectifier provides a pulsed DC signal to drive the deposition process.

The conditions of the electrochemical deposition process are preferably as illustrated below in Table III.

TABLE III

| Component                             | Preferred | More Preferred | Most Preferred |
|---------------------------------------|-----------|----------------|----------------|
| pH                                    | 12-14     | 12-13          | 12.5-13        |
| Temperature (°C.)                     | 5-30      | 10-25          | 10-20          |
| Time (minutes)                        | 5-80      | 15-60          | 20-30          |
| Current Density (mA/cm <sup>2</sup> ) | 2-90      | 5-70           | 10-50          |

These reaction conditions allow the formation of a ceramic-like coating of up to about 40 microns in about 80 minutes or less. Maintaining the voltage differential for longer periods of time will allow for the deposition of thicker coatings. However, for most practical purposes, coatings of about 10 to 30 microns in thickness are preferred and can be obtained through a coating time of about 10 to 30 minutes.

Coatings produced according to the above-described process are ceramic-like and have excellent corrosion and abrasion resistance and hardness characteristics. While not wishing to be held to this theory, it appears that these properties are the result of the morphology and adhesion of the coating on the metal substrate. The preferred coatings

comprise a mixture of fused silicon oxide and fluoride along with an alkali metal oxide.

The adhesion of the coating of the invention appears to perform considerably better than any known commercial coatings. This is a result of a coherent interface between the metal substrate and the coating. By coherent interface, it is meant that the interface comprises a continuum of magnesium, magnesium fluorides, magnesium oxides, magnesium oxofluorides and silicon oxides.

The continuous interface is shown in FIG. 4, a scanning electron photomicrograph. The metal substrate 50 has an irregular surface, and an interfacial boundary comprising a fluoride-containing base layer 52 is formed at the surface of the substrate 50. The magnesium oxide/silicon oxide-containing layer 54 becomes an integral part of the base layer 52. The combined layers 52 and 54 show excellent integrity, and therefore provide a superior corrosion and abrasion resistant surface. Abrasion resistance can be measured according to Federal Test Method Std. No. 141C, Method 6192.1. Preferably, coatings produced according to the invention having a thickness of 0.5 to 1.0 mil will withstand at least about 1,000 wear cycles before the appearance of the bare metal substrate using a 1.0 kg load on a CS-17 abrading wheel. More preferably, the coatings will withstand at least about 2,000 wear cycles before the appearance of the metal substrate, and most preferably, the coatings will withstand at least about 4,000 wear cycles using a 1.0 kg load on a CS-17 abrading wheel.

Corrosion resistance can be measured according to ASTM standards. Included in these tests is the salt fog test, ASTM B117, as evaluated by ASTM D1654, procedures A and B. Preferably, as measured according to procedure B, coatings produced according to the invention achieve a rating of at least about 9 after 24 hours in salt fog. More preferably, the coatings achieve a rating of at least about 9 after 100 hours, and most preferably, at least about 9 after 200 hours in salt fog.

After the magnesium-containing articles have been coated according to the present process, they may be used as is, offering a superb finish and excellent corrosion resistant properties, or they may be further coated using an optional finish coating such as a paint or a sealant. The structure and morphology of the magnesium oxide- and silicon oxide-containing coating readily permit the use of a wide number of additional finish coatings which offer further corrosion resistance or decorative properties to the magnesium containing articles. Indeed, the magnesium oxide- and silicon oxide-containing coating provides an excellent paint base having excellent corrosion resistance and offering excellent adhesion under both wet and dry conditions, for instance, the water immersion test, ASTM D3359, test method B. The optional finish coatings may include organic and inorganic compositions as well as paints and other decorative and protective organic coatings. Any paint which adheres well to glassy and metallic surfaces may be used as the optional finish coating. Representative, non-limiting inorganic compositions for use as an outer coating include additional alkali metal silicates, phosphates, borates, molybdates and vanadates. Representative, non-limiting organic outer coatings include polymers such as polyfluoroethylene, polyurethane and polyglycol. Additional finish coating materials will be

known to those skilled in the art. Again, these optional finish coatings are not necessary to obtain excellent corrosion resistance, their use may achieve decorative or further improve the protective qualities of the coating.

Excellent corrosion resistance occurs after further application of an optional finish coating. Preferably, as measured according to procedure B, coatings produced according to the invention, having an optional finish coating, achieve a rating of at least about 8 after 700 hours in salt fog. More preferably, the coatings achieve a rating of at least about 9 after 700 hours, and most preferably, at least about 10 after 700 hours in salt fog.

### EXAMPLES

The following specific examples, which contain the best mode, can be used to further illustrate the invention. These examples are merely illustrative of the invention and do not limit its scope.

#### Example I

Magnesium test panels (AZ91D) were cleaned immersing them in an aqueous solution of sodium pyrophosphate, sodium borate and sodium fluoride at about 70° C. and a pH

### 8 Examples II-VIII

Examples II-VIII were prepared according to the process of Example I with the quantities of components as shown in Tables IV and V below.

TABLE IV

| Example | Chemical Bath                             |                    |                            |
|---------|-------------------------------------------|--------------------|----------------------------|
|         | NH <sub>4</sub> F<br>Concentration<br>(M) | Bath Time<br>(°C.) | Residence<br>Time<br>(min) |
| II      | 1.0                                       | 70                 | 30                         |
| III     | 1.5                                       | 60                 | 30                         |
| IV      | 0.7                                       | 80                 | 30                         |
| V       | 1.0                                       | 80                 | 20                         |
| VI      | 1.0                                       | 70                 | 30                         |
| VII     | 0.8                                       | 80                 | 40                         |
| VIII    | 1.2                                       | 60                 | 30                         |

20

15

25

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

20

observed.

The foregoing description, Examples and data are illustrative of the invention described herein, and they should not be used to unduly limit the scope of the invention or the claims. Since many embodiments and variations can be made while remaining within the spirit and scope of the invention, the invention resides wholly in the claims hereinafter appended.

What is claimed is:

1. A magnesium-containing article offering improved corrosion and abrasion resistance, the article comprising a

magnesium-containing substrate coated with a first layer containing a continuum of magnesium fluoride, magnesium oxide, magnesium oxofluoride and silicon oxide.

5 2. The article of claim 1 further comprising a second, sealing layer disposed upon the layer.

3. The article of claim 2 further comprising a third, finish layer disposed upon the second, sealing layer.

10 4. The article of claim 1 which is substantially free of chromium (VI).

\* \* \* \* \*

UNITED STATES PATENT AND TRADEMARK OFFICE  
CERTIFICATE OF CORRECTION

PATENT NO. : 5,470,664

DATED : November 18, 1995

INVENTOR(S) : Bartak, et al.

It is certified that error appears in the above-identified patent and that said Letters Patent is hereby corrected as shown below:

ON THE TITLE PAGE:

Item [75], Line Inventors, "E. Grand Forks," should read --Baxter,--.

Item [73], Line Assignee, insert -Inc.-- after the word "Group,"

Signed and Sealed this  
Second Day of April, 1996

Attest:



BRUCE LEHMAN

Attesting Officer

Commissioner of Patents and Trademarks